

2,900,217

**PROCESS FOR DYEING PRODUCTS OF COPOLYMERS OF ACRYLONITRILE**

Hendrik Wanen, Nimeguen, Netherlands, assignor to Naamlooze Vennootschap Kunstzijdespinnerij Nyma, Nimeguen, Netherlands, a Dutch company

No Drawing. Application July 6, 1955  
Serial No. 520,355

Claims priority, application Netherlands July 16, 1954

1 Claim. (Cl. 8—42)

The invention relates to a process for dyeing products of copolymers of acrylonitrile, particularly those which contain more than 80% of acrylonitrile. The properties of such products are in general very similar to those of pure polyacrylonitrile: they excel because of their great strength, resistance to chemical attack and the action of light. They have, however, the drawback that they are difficult to dissolve—special solvents, for instance dimethyl formamide are necessary—and that they are very difficult to dye.

"Irgalan," "Neolan," "Cibalan," and "Palatin-echt" dyestuffs are known as acid wool dyestuffs which contain a complex bound metal, such as chromium or cobalt. Those dyestuffs do not dye polyacrylonitrile and the above-mentioned copolymers of acrylonitrile if one proceeds according to the procedure usual for wool, in which one acidifies the dye bath with acetic acid or  $(\text{NH}_4)_2\text{SO}_4$  and dyes at about 100° C.

"Neolan" and "Palatin-echt" are trademarks for 1-1 monoazo chromium dyes, existing under one or more of the following Colour Index numbers:

| "Neolan" |       | "Palatin-echt" |       |       |
|----------|-------|----------------|-------|-------|
| 13361    | 16260 | 13361          | 15685 | 18745 |
| 13425    | 16711 | 13420          | 16691 | 18900 |
| 13900    | 18736 | 13425          | 15708 | 18810 |
| 14006    | 18745 | 13900          | 15711 | 18870 |
| 14885    | 18800 | 14006          | 16055 | 19010 |
| 15050    | 18810 | 14251          | 16260 | 19065 |
| 15685    | 18870 | 14880          | 16265 | 19080 |
| 15691    | 19010 | 14885          | 16711 | 19115 |
| 15711    | 19115 | 14980          | 16760 | 19351 |
| 10055    | 19320 | 15025          | 18736 | 19355 |
|          | 19351 | 15680          | 18740 |       |

"Irgalan" and "Cibalan" are trademarks for metalliferous azo dyes without sulfonic acid groups and having two molecules of dyestuff per molecule of metal, these dyes being used in a substantially neutral dye bath and existing under one or more of the following Colour Index prototype numbers:

| "Irgalan" |      | "Cibalan" |      |      |
|-----------|------|-----------|------|------|
| 1050      | 1227 | 1051      | 1222 | 1325 |
| 1088      | 1302 | 1089      | 1223 | 1336 |
| 1183      | 1346 | 1179      | 1224 | 1337 |
| 1184      | 1347 | 1180      | 1303 | 1398 |
| 1225      | 1348 | 1181      | 1304 | 1399 |
| 1226      | 1397 |           |      |      |
|           | 1400 |           |      |      |

Other nitrogen-containing material than wool, such as nylon can be dyed with this type of dyestuffs, also in a weakly acidic medium at a temperature of about 100° C.

The latter is described in Example 2 of U.S.P. 2,674,515. It has now surprisingly been found that copolymers of acrylonitrile can be dyed with acid dyestuffs which contain a complex bound metal in the presence of a salt in the dye bath and a temperature of the dye bath of above 100° C.

French Patent No. 954,752 describes the dyeing of textile products of a copolymer of acrylonitrile and a vinyl halide, in which a temperature above 100° C. is used and in which a salt such as sodium phosphate is present. This patent relates to copolymers which are easily dissolved in ordinary solvents, such as acetone and which—parallel with their better solubility—absorb dyestuffs more readily. The dyeing process given in this patent, in so far as it relates to normal acid dyestuffs, is, therefore, entirely unsuitable for dyeing the difficultly soluble copolymers. That those copolymers can be dyed by choosing the temperature above 100° C. and in the presence of a salt, provided one makes use of acid dyestuffs which contain a complex bound metal, could not at all be expected on account of the knowledge provided by the cited French patent.

The invention is elucidated by the following examples.

*Example I*

20 400 grams of yarn of a copolymer of acrylonitrile (95%) and methyl methacrylate were dyed for one hour at 125° C. in a bath having the following composition: 7250 cm.<sup>3</sup> of water, 10 grams of Irgalan Red 3 G.

25 In this way a very pale color was obtained. When the same experiment was repeated, in which 75 grams of  $\text{Na}_2\text{SO}_4$  were added to the bath, a dark red yarn was obtained. The same improvement in the dyeing quality by the  $\text{Na}_2\text{SO}_4$  addition was established with Irgalan Gray BL and Irgalan Brown 3 BL.

Similar experiments in which  $\text{NaCl}$  or  $\text{NaCNS}$  was used instead of  $\text{Na}_2\text{SO}_4$  and in which a copolymer of acrylonitrile (95%) and of methyl acrylate or a copolymer of acrylonitrile (95%) and of vinyl acetate was dyed, proved the same favorable influence of the salt addition.

On repetition of all the above mentioned experiments, in which in the presence of a salt a dye temperature of 40 100° C. was chosen, no dyeing was obtained or a very pale dyeing was obtained.

*Example II*

45 400 grams of yarn of a copolymer of acrylonitrile (95%) and of methyl acrylate were dyed for one hour at 125° C. in a bath having the following composition: 7250 cm.<sup>3</sup> of water, 10 grams of Cibalan Yellow GRL, 75 grams of  $\text{NaCl}$ .

50 In this manner a clear yellow yarn was obtained. If experiment was repeated, in which no salt was added and/or the dye temperature of 100° C. was chosen, a pale yarn was obtained.

Similar experiments with the same dyestuff, in which 55 instead of yarn of the above mentioned copolymer yarn of a copolymer of acrylonitrile (95%) and of vinyl acetate or a copolymer of acrylonitrile (95%) and of methyl methacrylate was dyed and in which instead of 75 grams of  $\text{NaCl}$  one of the other salts mentioned in

60 Example I was used, proved the same favorable influence of the salt addition and the dye temperature of 125° C.

The invention is not concerned with those copolymers of acrylonitrile, for instance a copolymer of acrylonitrile and of vinyl pyridine, in which basic groups are introduced into the macromolecule which render it possible to dye the copolymer with acid wool dyestuffs by means of the basic group with the dyeing procedure usual for wool.

65 70 What is claimed is:

Process for dyeing a copolymer of acrylonitrile and an olefinic compound selected from the group consisting

of methyl acrylate, methyl methacrylate and vinyl acetate, which copolymer contains at least 80% of acrylonitrile, which comprises the step of treating the copolymer in a dye bath containing a metallized azo dyestuff selected from the group consisting of 1-1 monoazo chromium complex dyes and metalliferous azo dyes without sulfonic acid groups having two molecules of dyestuff per molecule of metal and used in a substantially neutral dye bath, and an inorganic water-soluble alkali salt at a temperature above 100° C.

## References Cited in the file of this patent

## UNITED STATES PATENTS

2,543,316 Feild ----- Feb. 27, 1951

## FOREIGN PATENTS

923,442 France ----- Feb. 17, 1947

## OTHER REFERENCES

10 Am. Dyestuff Reporter for Jan. 22, 1951, p. P51.